

## UNITED STATES PATENT OFFICE

GUSTAV SCHREIBER, OF BITTERFELD, GERMANY, ASSIGNOR, BY MESNE ASSIGNMENTS,  
TO MAGNESIUM DEVELOPMENT CORPORATION, A CORPORATION OF DELAWARE

PROCESS OF WORKING MAGNESIUM AND HIGH PERCENTAGE MAGNESIUM ALLOYS  
BY ROLLING

No Drawing. Application filed December 10, 1931, Serial No. 580,220, and in Germany December 16, 1930.

The present invention relates to an improved process of working magnesium and high percentage magnesium alloys by rolling.

5 It has been observed that in rolling magnesium and high percentage magnesium alloys certain difficulties appear which do not occur in the rolling of other metals, such as copper, brass, and aluminium. Whereas, 10 with the latter metals it is generally possible to start from cast bars (ingots) and to roll them down, in a more or less continuous manner, with considerable reduction in each pass, into plates or thin rods of any convenient 15 gauge, it has been found that, in rolling down cast magnesium, or cast high percentage magnesium alloys, even at the high working temperatures which are always necessary when working these metals, failure of the 20 material soon occurs by splitting or cracking. Hitherto, the only means of preventing such failure—and even that but inadequately—consisted in restricting the reduction in thickness by each pass to a relatively 25 low value, generally with interposed reheating, particularly in the early stages of rolling. Apparently a process of rolling magnesium and high percentage magnesium alloys, when carried on in this manner, is 30 hardly practicable on an economical basis.

An object of the present invention, therefore, is to obviate the aforementioned difficulties. I have ascertained that the cracking and splitting of the cast material under the stresses exercised by the rolling mill is largely due to the always comparatively coarse-grained structure of the cast material, the coherence of the individual crystals being insufficient to withstand the high specific stresses of rolling which are concentrated over an extremely narrow portion of the boundary surfaces of the material. It would appear therefrom that it is necessary to improve the grain of the cast material by refining it preliminary to subjecting it to the action of the rolling mill, in order to obviate the drawbacks of the former process.

According to the present invention the refining of the grain of the cast material is

effected by subjecting the material, prior to rolling, to a plastic deformation at high temperatures by the application of specific pressures which are moderate as compared with those exercised by a rolling mill, and which are further distinguished from the latter by acting on a considerable portion of the boundary surfaces of the material. Such plastic deformation is preferably effected by means of an extrusion press, or by forging, 55 and at the temperatures which are customary in the working of magnesium and high percentage magnesium alloys by these processes. At the same time, in view of the shaping aimed at by the subsequent rolling mill treatment, it is advisable to combine the preliminary kneading action on the cast material with a molding action which, to a greater or lesser extent, anticipates the further shaping of the material by rolling. For example, 60 if rolled plates are to be produced, a cast ingot is first transformed in an extrusion press, in the manner known per se, into a section of flat rectangular shape (flat bar) which is subsequently subjected to the rolling process, 65 advantageously in the same heat.

*Example*

A cast cylindrical block of 800 mm. length and 170 mm. diameter of an alloy containing approximately 6 percent of aluminium, about 1 percent of zinc, and traces of manganese, the balance being magnesium, is extruded into a flat rectangular section of 240 mm. x 20 mm. cross-section, at a temperature of about 380° C., which is the customary temperature of extruding an alloy of that composition. The extruded section, if necessary after reheating, is subjected to rolling 80 in the following manner:

The rolling is carried out in pairs of passes, each pair followed by reheating to a temperature slightly higher than that applied to the material prior to the preceding pair 85 of passes, in such a manner that rolling begins at 340° C. and is completed at 380° C. The decrease in thickness is about 10 to 12 percent of the actual thickness in each pass, down to a thickness of the sheets of about 3 90 100

mm., and about 5 to 8 percent below 3 mm. thickness down to 1 mm.

In the manner described the marketable crude products such as thin plate and the like, can be turned out without any special difficulty since the pretreated rolling material flows between the rolls in a far readier and more uniform manner than the cast material.

I claim:

- 10 1. A process of producing rolled articles from magnesium and high percentage magnesium alloys, which comprises subjecting the metal as cast to a plastic deformation by the application of specific pressures which are moderate as compared with those exercised by a rolling mill, and which act on a considerable portion of the boundary surfaces of the cast metal, and then rolling such deformed metal.
- 15 2. A process of producing rolled articles from magnesium and high percentage magnesium alloys, which comprises subjecting the metal as cast to a plastic deformation by forging, and then rolling such deformed metal.
- 20 3. A process of producing rolled articles from magnesium and high percentage magnesium alloys, which comprises subjecting the metal as cast to a plastic deformation by extruding and then rolling such deformed metal.
- 25 4. A process of producing rolled articles from magnesium and high percentage magnesium alloys, which comprises subjecting the metal as cast to a plastic deformation by extruding, and then repeatedly subjecting such deformed metal to rolling at temperatures which are successively the higher the thinner the work-piece is rolled out.
- 30 5. A process of producing rolled articles from magnesium and high percentage magnesium alloys, which comprises subjecting the metal as cast to a plastic deformation by extruding the metal into a section of flat rectangular shape, and then rolling such deformed metal.
- 35 6. A process of producing rolled sheets from an alloy consisting of about 6 percent of aluminium, about 1 percent of zinc, traces of manganese, the balance substantially being magnesium, which comprises extruding such metal alloy as cast into a section of flat rectangular shape at a temperature of about 380° C., and then repeatedly subjecting such extruded section to rolling at temperatures successively increasing from about 340° C. to about 380° C.

In testimony whereof, I affix my signature.  
GUSTAV SCHREIBER.

## DISCLAIMER

1,902,905.—*Gustav Schreiber*, Bitterfeld, Germany. PROCESS OF WORKING MAGNESIUM AND HIGH PERCENTAGE MAGNESIUM ALLOYS BY ROLLING. Patent dated March 28, 1933. Disclaimer filed May 26, 1934, by the assignee, *Magnesium Development Corporation*, with *I. G. Farbenindustrie Aktiengesellschaft* assenting and joining.

Therefore, enters this disclaimer to certain of the claims of the above identified patent, and

Hereby disclaims claims 3 and 5.

Hereby disclaims from the scope of claim 1 any process in which the step of subjecting the metal as cast to a plastic deformation is accomplished by extrusion.

[*Official Gazette June 19, 1934.*]